

June 18, 1929.

C. T. DRAPER

1,718,039

METHOD OF PROTECTIVELY COATING CONTAINERS

Filed Feb. 5, 1925

2 Sheets-Sheet 1



INVENTOR:  
CHARLES T. DRAPER  
  
ATTORNEY

June 18, 1929.

C. T. DRAPER

1,718,039

METHOD OF PROTECTIVELY COATING CONTAINERS

Filed Feb. 5, 1925

2 Sheets-Sheet 2



FIG. 7.



INVENTOR:  
CHARLES T. DRAPER

*Charles T. Draper*  
ATTORNEY

Patented June 18, 1929.

1,718,039

# UNITED STATES PATENT OFFICE.

CHARLES T. DRAPER, OF CLEVELAND, OHIO, ASSIGNOR TO THE DRAPER MANUFACTURING COMPANY, OF CLEVELAND, OHIO, A CORPORATION OF OHIO.

## METHOD OF PROTECTIVELY COATING CONTAINERS.

Application filed February 5, 1925. Serial No. 7,075.

My invention relates to improvements in method of protectively coating sheet metal containers, and has for its object a procedure whereby the surfaces, and, more particularly, the interior surface of the container may cheaply, evenly and expeditiously be provided with a suitable protective coating.

Sheet metal containers previously have been interiorly coated by introducing the protective material in heated, liquid or finely subdivided condition; the latter by spraying the liquid. However, these methods do not lend themselves to an even and accurate distribution of the coating material throughout the interior of a container and it frequently is the common practice to make duplicate or triple applications of the material in order measurably to insure a complete covering of the surfaces. Frequently, as with barrels and drums formed of sheet metal, this coverage merely is assumed, since the operative cannot visually assure himself of any complete application of the protective coating, while uneven distribution and unnecessary expense almost certainly are involved through practicing the prior methods.

Accordingly, I have devised an improved method for protectively coating various classes of sheet metal containers by introducing a quantity of suitable coating substance that is rendered fluid upon heating the container; meanwhile rotating the heated container to insure distribution of the liquefied substance evenly over its interior surfaces. In order to insure the even and economical coverage of all interior surfaces and seams, it is found desirable to apply the coating material to the blanks from which the container is fabricated before they are seamed together; all as will be more fully explained in the accompanying specification and claims, having particular reference to the drawings, wherein:

Figure 1 is a perspective view of the cylindrical shell for forming a sheet metal drum,

Fig. 2 is a similar view of a head therefor, Fig. 3 is a fragmentary sectional view upon an enlarged scale illustrating the evenly applied interior coating,

Fig. 4 is a diagrammatic plan view of apparatus adapted for practicing my improved method,

Fig. 5 is a longitudinal sectional view thereof on line V—V, Fig. 4,

Fig. 6 is an enlarged cross sectional view on line VI—VI, Fig. 5, and

Fig. 7 is a fragmentary longitudinal section upon an enlarged scale on line VII—VII, Fig. 6.

Throughout the several figures of the drawings I have employed the same character of reference to indicate similar parts.

Suitable protective coating materials vary widely with the particular use and proposed contents of the sheet metal container, comprising such materials as paraffin, wax, shellac and gums of various sorts. In fact, any suitable protective material or substance which becomes liquid or vaporous with the application of moderate heat and which can readily be dried or solidified by cooling is one lending itself to the instant method. Nevertheless, I may sufficiently explain my invention by describing the application of a paraffin coating, preferably distributed over areas of the blanks prior to seaming them and testing the completed drum.

The sheet metal drum *a*, shown in completed form in Figs. 3, 6 and 7, may be taken as typical of any sheet metal container; comprising in this instance the cylindrical shell *a'* and the heads *a''* that are seamed together in the well known manner to produce a liquid-tight container. These members or blanks may have adequate quantities of coating material applied thereto in distributed areas, as *c*, *c'*, respectively applied to the body portion and to the heads as shown. We may assume that the desired coating is paraffin, which may be applied in liquid form promptly solidifying in irregular form when brought in contact with the metal. The drum thereupon is suitably seamed circumferentially of the heads, as shown in Fig. 6, whereupon it may be subjected to the usual tests before the coating is distributed.

On the other hand, it may be found desirable to introduce the coating substance after the completion and testing of the sheet metal container, which may be done through the opening *b* provided with the usual screw-closure member *b'*. The coating substance may be sprayed through said opening, or it may be melted and poured into the container according to its characteristics and fully in accordance with the spirit and intent of my

present invention. It may be observed here that when substances volatilizing at relatively low temperatures are employed for the coating material, it is necessary to insert 5 the closure member *b'* in the opening, and frequently this is desirable during the heating period, in any case, in order to safeguard the coating material and prevent the entrance of foreign substances.

10 In my application, Ser. No. 728,535, July 28th, 1924, I have shown apparatus, partly reproduced in the accompanying drawings, adapted for practicing my present improvement, although I wish it to be understood 15 that the same is quite independent of the means for accomplishing the procedure and method hereinafter claimed.

Referring then to the second sheet of drawings, an elongated tunnel *d* is diagrammatically shown in Fig. 4 equipped with heaters *e*, *e* adapted to direct currents of heated air in both directions intermediately of said tunnel. A loading station and platform *f* appear upon the right, while the coated 25 containers *a*, *a* are removed from the conveyor *g* after passing beyond the tunnel and after being cooled. The details of the traveling conveyor *g* may be explained by referring to Figs. 6 and 7 wherein the supporting 30 rails *h* are engaged by the chime of the container, while rollers *i*, provided upon the upper pass of the linked conveyor *j*, serve slowly to advance the containers by rolling them along the rails from one end of the 35 heated tunnel to the other. L-shaped rails *k* serve to support the lower or returning section of the linked conveyor; the respective movements thereof and of the rotated containers being indicated by darts, Fig. 7.

40 Quite obviously the degree of heat to which the containers shall be subjected is governed primarily by the character of the coating material; paraffin, herein assumed for the purpose of illustration, melting and 45 flowing freely approximately at 150° F. Accordingly, the liquid coating material, as paraffin, will readily flow over the surfaces of the heads and interiorly of the body of the container as it is rolled through the 50 heated tunnel, thereby evenly distributing the coating material over the surfaces of the metal, where it will remain upon permitting the container to cool exteriorly of the tunnel and during rotation thereof. Thus the 55 containers may very expeditiously and cheaply be provided with an interior protective coating that is certain to cover all of the surfaces and seams interiorly thereof, simply by availing of the expedient of rolling the con-

tainers with the introduced coating material, 60 first in heated condition and thereafter cooling them in order to fix the distributed coating material in place.

As explained, I do not limit myself to the apparatus disclosed, nor to the particular 65 procedure above outlined for rotating, heating and cooling the treated containers, except as defined in the appended claims.

Having now described the practice of my invention in its preferred mode or manner, I 70 claim as new and desire to secure by Letters Patent, the following:

1. The herein described method of applying an interior coating to sheet metal containers, which consists in applying a quantity of a substance that is solid at normal temperatures and fluid at higher temperatures to the inner surface of the blank, completing the sheet metal container, heating said container and the contained substance 80 sufficiently to render the latter fluid, rotating said container, and permitting it to cool after the substance has been evenly distributed over the interior surfaces of the container, substantially as set forth. 85

2. The herein described method of applying an interior protective coating to sheet metal barrels and drums, which consists in placing sufficient quantities of a substance that is solid at normal temperatures and fluid 90 at higher temperatures upon the inner surfaces of the heads and body blank, seaming and testing the sheet metal container, heating said container sufficiently to render the coating substance fluid, rotating the container in heated condition, and permitting it to cool after the coating has been evenly distributed over the interior surfaces of the container, substantially as set forth. 95

3. The herein described method of applying an interior protective coating to sheet metal barrels and drums, which consists in distributing approximately the required quantities of a substance that is solid at normal temperatures and fluid at higher 105 temperatures upon the inner surfaces of the heads and shell in adjacent covering positions, seaming the sheet metal container, heating said container sufficiently to render the coating substance fluid, rotating the container in heated condition and permitting it to cool initially while rotating after the coating has been evenly distributed over the interior surfaces of the container, substantially as set forth. 110 115

In testimony whereof I do now affix my signature.

CHARLES T. DRAPER.